

Patented May 5, 1925.

## UNITED STATES PATENT OFFICE.

VERE B. BROWNE, OF BRACKENRIDGE, PENNSYLVANIA, ASSIGNOR TO VALLEY HOLDING CORPORATION, OF BRACKENRIDGE, PENNSYLVANIA, A CORPORATION OF PENNSYLVANIA.

## METHOD OF MANUFACTURING STEEL SHEETS.

No Drawing.

Application filed October 13, 1924. Serial No. 743,498.

*To all whom it may concern:*

Be it known that I, VERE B. BROWNE, a citizen of the United States, and a resident of Brackenridge, in the county of Allegheny and the State of Pennsylvania, have made a new and useful Invention in Method of Manufacturing Steel Sheets, of which the following is a specification.

This invention relates to the manufacture of stamping steel, and particularly to the manufacture of high-grade steel sheets for use in automobile, metal furniture and other trades where steel sheets having a highly finished surface and suitable for 10 deep and difficult stamping operations are required.

An object of this invention is to provide a method whereby high-grade steel sheets; that is, sheets free from Stead's brittleness 20 and having a smooth surface, may be uniformly manufactured with the standard sheet mill equipment.

This, as well as other objects which will readily appear to those skilled in this particular art, I attain by means of the method described in the specification and set forth in the appended claims.

In carrying out this method, sheet bars of the proper thickness and length are heated 30 to rolling temperature and rolled or broken down to approximately sixty per cent of the length of the sheets required. These semi-finished sheets or breakdowns are then annealed, pickled to remove the scale and 35 cold rolled to an extent necessary to eliminate all superficial surface defects formed during the hot rolling.

The sheets, after being subjected to this step of cold rolling, are matched, heated to 40 a temperature suitable for rolling but low enough to avoid scaling, and are rolled to the length required. This hot-rolling operation is carried on on a mill having highly polished smooth rolls.

45 The sheets after this hot-rolling operation are then annealed, pickled and finished in the regular way.

Since the surface of the sheets is smooth

and free from defects due to the final hot-rolling on a mill having smooth highly-polished rolls, it is not necessary to resort to cold rolling in the finishing operation, and the omission of cold rolling during the finishing operation avoids the occurrence of Stead's brittleness in the final anneal. 50 55

I find that, by means of this method, I am able to produce sheets of uniformly high-grade surface and suitable for deep drawing and stamping operations.

Having thus described my invention, 60 what I claim is:—

1. The method, which consists in hot-rolling sheet bars to approximately sixty per cent of the finished length of the sheets required, then in annealing and pickling the semi-finished sheets, then in cold rolling the same to an extent necessary to remove superficial surface defects, then in matching and heating the same to a relatively low temperature, then in rolling the match sheets 65 to length between highly polished smooth rolls and then in annealing and pickling the sheets whereby steel sheets having a high-grade surface and suitable for deep drawing and stamping operations are produced. 70 75

2. The method, which consists in breaking down sheet bars to approximately sixty per cent of the finished length of the sheets required, then in annealing the breakdowns, then in removing the scale by pickling, then 80 in removing superficial surface defects by cold rolling, then in matching and heating the break-downs to a temperature suitable for rolling, but not high enough to produce scaling, then in rolling the break-downs to 85 length between highly polished smooth rolls, then annealing the sheets and then in pickling the same whereby steel sheets having a high-grade surface and suitable for deep drawing and stamping operations are 90 produced.

In testimony whereof, I have hereunto subscribed my name this 8th day of October, 1924.

VERE B. BROWNE.